# EUROPEAN PATENT SPECIFICATION

(11) **EP 0 515 388 B1**
(45) Date of publication and mention of the grant of the patent: **18.11.1993**
(21) Application number: 91902089.1
(22) Date of filing: 12.01.1991
(51) Int. Cl.: G03C 1/34, G03C 7/392

(54) **PHOTOGRAPHIC SILVER HALIDE MATERIALS CONTAINING A STABILISER COMPOUND**
STABILISATORVERBINDUNG ENTHALTENDE PHOTOGRAPHISCHE SILBERHALOGENIDMATERIALIEN
MATERIAUX PHOTOGRAPHIQUES A L'HALOGENURE D'ARGENT CONTENANT UN COMPOSE DE STABILISATION

(30) Priority: 23.01.1990 GB 9001487
(43) Date of publication of application: 02.12.1992
(73) Proprietor: KODAK LIMITED, Harrow, Middlesex HA1 4TY (GB); EASTMAN KODAK COMPANY, Rochester, New York 14650-2201 (US)
(72) Inventor: LEYSHON, Llewellyn, James, c/o Kodak Ltd, Harrow, Middlesex, HA1 4TY (GB); SIDHU, Jasbir, c/o Kodak Ltd, Harrow, Middlesex, HA1 4TY (GB)
(74) Representative: Baron, Paul Alexander Clifford
(86) International application number: EP9100068
(87) International publication number: WO9111749

(56) References cited:
- JP-A-61 158 331
- US-A- 4 155 765
- US-A- 4 254 216
- US-A- 4 623 617
- US-A- 4 863 842
- US-A- 4 906 559

## Description

This invention relates to photographic silver halide materials containing a stabiliser compound and particularly to colour photographic materials.

US Patent 3 591 381 describes the use of 6-chromanols as stabilisers for azo dyes, reducing fade caused by light, moisture and heat. US patent 4 155 765 describes O-substituted 6-chromanols used as photographic dye image stabilisers. JP-A-61 158 331 describes the use of 8-chromanols to provide magenta dyes of improved light fastness with certain bicyclic magenta couplers. US-A-4 863 842 and US-A-4 623 617 have similar scope except that they concern 7-chromanols.

The present invention employs 7-chromanols as stabilisers in photographic materials containing yellow couplers which can form azomethine image dyes. It has been found that not all chromanol-coupler combinations have the same properties, for example 6-chromanols have a deleterious effect on image dye stability when used in combination with yellow couplers.

According to the present invention there is provided a colour photographic material comprising a support carrying at least one photographic silver halide emulsion layer having associated therewith a yellow dye-forming colour coupler and a 7-chromanol having the general formula:
wherein
R¹ is H, alkyl, substituted alkyl (including arylalkyl), or -R⁸-COOR,
R is an alkyl,
R² - R⁶ are each, independently, H or an alkyl group, and
R⁸ is an alkylene group.

In a preferred embodiment, the present photographic materials have incorporated therein a dye-forming colour coupler. Such couplers are well known and are often incorporated in photographic materials as a dispersion in droplets of a coupler solvent.

Examples of chromanol compounds useful in the present invention are listed in the following Table.

The chromanols and O-substituted-chromanols employed in the present invention may be prepared by reaction of the appropriate dihydric phenol with the appropriate diene, eg 2,5-dimethyl-2,4-hexadiene to form the basic chromanol followed by other reactions, in themselves known, to introduce a further substituents. Such processes are illustrated in Examples below.

The chromanols are used in an amount sufficient to stabilize the photographic image dyes and their precursors e.g. in an amount from 0.2 to 2.0 mole per mole coupler, more preferably at approximately equimolar amounts.

The chromanol may be incorporated in the silver halide emulsion layer or a layer adjacent thereto. It can be incorporated as a separate dispersion, but is preferably incorporated in admixture with the coupler. Both coupler and stabilizer may be dissolved in a conventional coupler solvent, such as dibutyl phthalate. As in the production of ordinary coupler dispersions, a volatile and/or water-miscible auxiliary solvent, such as ethyl acetate, may be used to aid the dispersion process and then removed by evaporation or by washing the set dispersion. Also, the dispersion process can be assisted by the presence of a surface active compound, as usual in the manufacture of coupler dispersions.

In the following discussion of suitable materials for use in the emulsions and elements of this invention, reference will be made to Research Disclosure, December 1978, Item 17643, published by Industrial Opportunities Ltd., The Old Harbourmaster's, 8 North Street, Emsworth, Hants P010 7DD, U.K., the disclosures of which are incorporated herein by reference. This publiciation will be identified hereafter as "Research Disclosure". References giving information on couplers and on methods for their dispersions are given in Sections VII and XIV, respectively, of Research Disclosure.

The yellow couplers which may employed in the present photographic materials are water-insoluble acylacetanilide compounds containing ballast groups. Patents describing yellow couplers for use in the present invention include the following United States Patents:

### Yellow dye-forming

2 298 443 3 277 155
2 407 210 3 408 194
2 875 057 3 415 652
2 908 573 3 447 928
3 265 506 3 933 501
An account of dye-forming development is given in 'Modern Photographic Processing', Vol. 2, Grant Haist, Wiley, New York, 1978, Chapter 9.

The stabilizers are useful in any coupler-incorporated silver halide photographic materials, including monochrome materials, false-colour materials and colour transparency, negative and print materials, to stabilize the image dye obtained on development with a solution including a p-phenylenediamine colour developing agent. Such developing agents are well-known, being described in,for example Photographic Processing Chemistry, L.F.A. Mason, Focal Press, London, 2nd edition (1975) pp 229-235 and Modern Photographic Processing, Grant, Haist, Wiley, New York (1979), Volume 2 pp 463-8. They may also be used in colour materials not containing couplers but processed in developer solutions containing couplers.

The silver halide emulsion employed in the elements of this invention can be either negative-working or positive-working. Suitable emulsions and their preparation are described in Research Disclosure Sections 1 and II and the publications cited therein. Suitable vehicles for the emulsion layers and other layers of elements of this invention are described in Research Disclosure Section IX and the publications cited therein.

The photographic elements of this invention or individual layers thereof, can contain brighteners (see Research Disclosure Section V), antifoggants and stabilizers (see Research Disclosure Section VI), antistain agents and image dye stabilizer (see Research Disclosure Section VII, paragraphs I and J), light absorbing and scattering materials (see Research Disclosure Section VIII), hardeners (see Research Disclosure Section XI), plasticizers and lubricants (see Research Disclosure Section XII), antistatic agents (see Research Disclosure Section XIII), matting agents (see Research Disclosure Section XVI) and development modifiers (see Research Disclosure Section XXI).

The photogaphic elements can be coated on a variety of supports as described in Research Disclosure Section XVII and the references described therein.

Photographic elements can be exposed to actinic radiation, typically in the visible region of the spectrum, to form a latent image as described in Research Disclosure Section XVIII and then processed to form a visible dye image as described in Research Disclosure Section XIX. Processing to form a visible dye image includes the step of contacting the element with a colour developing agent to reduce developable silver halide and oxidize the colour developing agent. Oxidized colour developing agent in turn reacts with the coupler to yield a dye.

With negative working silver halide emulsions this processing step leads to a negative image. To obtain a positive (or reversal) image, this step can be preceded by development with a non-chromogenic developing agent to develop exposed silver halide, but not form dye, and then uniform fogging of the element to render unexposed silver halide developable. Alternatively, a direct positive emulsion can be employed to obtain a positive image.

Development is followed by the conventional steps of bleaching, fixing, or bleach-fixing, to remove silver and silver halide, washing and drying.

The following Examples are given for a better understanding of the invention.

### EXAMPLE 1

### Preparation of 2,2-dimethyl-4-isopropyl-7-hydroxy-3,4-dihydro-benzopyran (6).

Resorcinol (11.0g, 0.1m), petroleum ether (b.p. 60-80°) (2ml) and orthophosphoric acid (5mls) were stirred at room temperature. To the stirred mixture 2,5-dimethyl-2,4-hexadiene (11.0g, 0.1m) was added dropwise (1/2 hr) keeping the temperature of the reaction mixture between 30-35°C. After refluxing the reaction for 8 hrs. it was poured into ice/water, extracted with ethyl acetate, dried and evaporated to dryness. The 7-chromanol (6) was obtained in 89% yield by column chromatography.

### EXAMPLE 2

### Preparation of 2,2-dimethyl-4-isopropyl-6-t-butyl-7-hydroxy-3,4-dihydrobenzopyran (7).

To a stirred mixture of the 7-chromanol (6) (4.38g, 0.2m) and t-butanol (10ml), sulphuric acid (5ml) was added dropwise keeping the temperature of the reaction mixture between 25-30°C. The reaction mixture was stirred at room temperature for 3 hrs, then poured onto ice/water. The solid was filtered and crystallised from aqueous ethanol to afford the butylated chromanol (7) (4.4g, 85%).

### EXAMPLE 3

### Preparation of 2,2-dimethyl-4-isopropyl-6-t-butyl-7-benzyloxy-3,4-dihydrobenzopyran (8).

To a stirred mixture of 7-chromanol (7), (5.5g, 0.2m) and potassium carbonate (5gms) in acetone (30ml), benzylbromide (3.42g, 0.2m) was added. The reaction mixture was refluxed with stirring for 18 hrs. The reaction mixture was poured onto ice/water, extracted with ethyl acetate, dried and evaporated to afford a lemon-yellow solid. Crystallisation from aqueous ethanol gave the required product (6.6g, 90%).

### EXAMPLE 4

### Yellow dye light stability improvement

Single layer film strips were prepared by coating a gel-subbed polyethylene-terephthalate support with a photosensitive layer containing a silver bromoiodide emulsion at 0.398 Ag/m², gelatin at 1.36g/m² and dispersion of coupler (9) in coupler solvent (10) (1.5 moles/mole of coupler). The coupler coverage was 0.83 millimoles/m². The photographic layer was overcoated with a layer containing gelatin at 3.0g/m² and bis-vinylsulphonylmethylether hardener at 1.5 weight percent based on total gelatin. Similar coatings were prepared using coupler dispersions which also contained one of the stabilisers (I) and (III) at 0.5 mole per mole coupler.

Samples were exposed through a graduated density test object and developed with 4-amino-3-methyl-N-ethyl-N-β-(methanesulphonamido)ethyl-aniline in an EP-2 process.

Patches from each coating having a density at or above 1.0 were faded for 6 weeks using a 5.4 klux xenon source, the UV component of which was removed by a coating of Tinuvin 328 (Trade Mark of Ciba-Geigy) in a gelatin dispersion at a coverage of 750 mg/m² on a transparent support. The loss in transmission optical density at the wavelngth of maximum absorption was measured. The data is presented below in Table 2.

The presence of Stabiliser compounds (I) and (V) greatly improved the fade performance in all cases.

### EXAMPLE 5 (Comparative)

In a comparative experiment, coatings were prepared as described in Example 4, except that the test materials included in the coupler dispersion were the 6-chromanols (Ia) and (Ib). The results of the fade experiments showed that these 6-chromanols greatly reduced the stability of the yellow image dye as shown in Table 3 below.
Compounds Ia and lb were as follows:

## Claims

1. A colour photographic material comprising a support carrying at least one photographic silver halide emulsion layer having associated therewith a yellow dye-forming colour coupler and a 7-chromanol image dye stabiliser having the general formula: wherein
R¹ is H, alkyl, substituted alkyl (including arylalkyl), or -R⁸-COOR,
R is an alkyl,
R² - R⁶ are each, independently, H or an alkyl group, and
R⁸ is an alkylene group,.

2. A photographic material as claimed in claim 1 in which the alkyl groups contain from 1-4 carbon atoms.

3. A photographic material as claimed in Claim 1 or 2 in which the chromanol is selected from one of the following:

## Patentansprüche

1. Farbphotographisches Material mit einem Träger, auf den mindestens eine photographische Silberhalogenidemulsionsschicht aufgetragen ist, der ein einen gelben Bildfarbstoff bildender Farbkuppler und ein 7-Chromanol-Bildfarbstoffstabilisator zugeordnet ist, der der folgenden allgemeinen Formel entspricht: worin bedeuten: R¹ gleich H, eine Alkylgruppe, eine substituierte Alkylgruppe (einschließlich einer Arylalkylgruppe), oder -R⁸-COOR,
R eine Alkylgruppe,
R² - R⁶ jeweils unabhängig voneinander H oder eine Alkylgruppe und
R⁸ eine Alkylengruppe.

2. Photographisches Material nach Anspruch 1, in dem die Alkylgruppen 1 bis 4 Kohlenstoffatome ausweisen.

3. Photographisches Material nach Anspruch 1 oder 2, in dem das Chromanol ausgewählt ist aus einem der folgenden Chromanole:

## Revendications

1. Matériau photographique en couleurs comprenant un support contenant au moins une couche d'émulsion photographique aux halogénures d'argent à laquelle est associé un coupleur formateur de colorant jaune et un stabilisateur d'image de colorant 7-chromanol de formule générale : où
R¹ est un hydrogène, un alkyle, un alkyle substitué (y compris arylalkyle), ou -R⁸-COOR,
R est un groupe alkyle
R² et R⁶ sont chacun, indépendamment, un hydrogène ou un groupe alkyle, et
R⁸ est un groupe alkylène.

2. Matériau photographique selon la revendication 1, dans lequel les groupes alkyles contiennent de 1 à 4 atomes de carbone.

3. Matériau photographique selon la revendication 1 ou 2, dans laquelle le chromanol a l'une des formules suivantes :
